

## UNITED STATES PATENT OFFICE

2,357,913

PHOTOGRAPHIC PROCESS FOR ETCHING  
FIGURES ON GLASS

John V. Sigford, Wabash, Ind., and Waldo H. Kliever, Minneapolis, Minn., assignors to Minneapolis-Honeywell Regulator Company, Minneapolis, Minn., a corporation of Delaware

No Drawing. Application August 29, 1941,  
Serial No. 408,818

1 Claim. (Cl. 95—5.7)

Our invention relates broadly to an improved process for etching whereby, in the etching of figures in material in general, the differential effects are obtained from differential exposure to light and the common methods of mechanically marking a resist are eliminated.

In particular, the invention relates to a new and novel photo-engraving process involving the etching of glass, quartz, vitreous enamel, plastics and other substances. A particular object of our invention is the provision of a process for the photo-engraving and etching of glass to be employed as reticles for use in telescopes, range finders, microscopes, surveying and other optical or aligning instruments. However, it will be obvious that our invention is of broad application in the fields of photo-etching and of photo-engraving and accordingly is to be limited only by the scope of the appended claim.

In well known photo-engraving processes such as those embodying the use of copper or zinc plates for printing, the configuration to be reproduced by etching is photographed for the making of negatives from which the etching resist pattern is produced on the metal. The metal is coated with a light sensitive colloid, exposed under the negative to a strong actinic light and treated to produce the enamel etching resist of a material such as insoluble glue or albumen. In the etching process the metal which is not protected is controllably dissolved by the action of the etching mordant while leaving the protected or enameled portions in relief. Well known etching mordants employed in connection with these metals may consist of ferric chloride for the copper and nitric acid for the zinc. In the usual methods for etching glass and optical material, an etching mordant such as hydrofluoric acid must be employed. It is found that such a mordant will attack light sensitive coatings even though it has been exposed and treated to form an enamel etching resist of the type successfully employed with metals. It is an object of this invention to provide a photo-etching and a photo-engraving process for etching in fine detail materials in general. A particular object of the invention is the provision of a process for the photo-etching of glass and like materials that require the use of an etching mordant such as hydrofluoric acid which is harmful to resists of the type normally employed in connection with known photo-engraving processes.

A further object of the invention is to provide a process for the photo-etching of materials which permits the use of an etching mordant

such as hydrofluoric acid which will attack a light sensitive resist by the use of a suitable resist in proper relation with the light sensitive material. For example, in accordance with our invention, the material to be etched may be coated with silver to form a suitable resist for a hydrofluoric acid etching mordant. The well known photo-engraving processes referred to above may then be employed. Thus the portions of bichromated colloid coating for the material when exposed to light under a suitable negative will become insoluble to form a suitable resist for an etching solution for silver or other first coating. The silver in the image which is not protected by the enamel of the resist may accordingly be dissolved away by immersion in a solution of sodium thiosulphate and potassium ferricyanide known as Farmer's reducer, or other mordant. When the image is thus obtained on the material proper, it is rinsed, dried and may then be etched by the hydrofluoric acid mordant. The material is then rinsed in concentrated nitric acid to remove any remaining enamel and silver to thus complete the etching process.

Other objects and advantages will become apparent to those skilled in the art and a more thorough understanding of our invention will be obtained by reference to the accompanying description of the application thereof to the production of reticles for use in telescopes and range finders.

In the practice of our invention as applied to the production of reticles in glass, the glass material must be treated in accordance with known processes to render it chemically clean. The glass is then silvered and this may be accomplished by the use of any standard process such as used in the making of mirrors including chemical deposition, cathodic sputtering, or by evaporation processes. The silvering may be accomplished with very good results by the use of the well known Rochelle salts process, and in order to produce a perfectly resistant coating it is preferable that at least three successive coatings be employed. It is found desirable to carry the silvering to a stage where it has a slightly white appearance which occurs after the solution has become sludgy. In this manner a surface is obtained to which the enamel will better adhere than is the case with a perfectly smooth coating, although if the surface is permitted to become too white the enamel described below would be porous and non-resistant.

In the handling of telescopic reticles a sheet 55 of plastic containing recesses for holding the

reticles in place may be employed. The cleaning and silvering may be accomplished by the use of trays such as used in photographic work. In this manner they may be handled in quantities of, for example, two hundred at a time. The cleaning and silvering operations may be performed in a period of about thirty minutes.

The silvered reticles are then coated with a light sensitive bichromated colloid film which when exposed under the negative, forms the etching resist for the silver etching process described below. The sensitizing solution may consist of sensitized resin which usually contains bichromate and is known in general as Cold Top enamel. Other colloidal substances employed may be of the fish glue type, gelatine, bone or hide glue, gum arabic and other known substances may be employed. The Cold Top enamel or sensitive glue coating solution is applied to the silvered reticles and preferably made to flow evenly by a centrifugal or spinning process. The reticle may be attached by a suction cup to a drill stock or motor which is rotated at a relatively low speed and the coating material is applied to the center of the reticle. It is desirable that the coating be applied as evenly as possible and the thickness of the coat should be controlled because of its effect on the exposure required. The thickness of the coat depends on the temperature and the speed of rotation. A light is employed that is not sufficiently bright for exposure purposes. The coating must be thin enough to give the desired detail and thick enough to provide the required resists.

The coating thickness may be instantly gaged without stopping the spinner by observing the interference pattern on the surface. We have found that the formation of a red interference disc of the first order in the center of the rotating reticle, when dry, is indicative of a thickness of one-half wave length of red light, or about 0.00003 inch. Two coats are preferred, the second being applied after the first has dried. It will be found that the coat will be smoother if the surface while spinning and before the coating is applied is lightly rubbed with a piece of cotton wet with alcohol. The coating process requires about three minutes and one person may conveniently handle about ten spinners at once.

The network and markings of the figure to be reproduced in glass as required in the formation of reticles for telescopes and range finders may be drawn on paper at preferably many times the actual size. In producing an accurate image in the negative it is necessary to so design the figure contained in the drawing as to compensate for lens imperfections and film halation by revision of the drawing in an amount determined by experimentation. The figure may then be copied on a process film or plate and then recopied on microfilm or some high resolution film, for example, by using a lens of short focal length possessing excellent resolving power to provide the necessary sharp and fine detail. To minimize halation, the exposure may be kept somewhat light with copper intensification employed to obtain sufficient density in the image. Our invention is not limited to the use of photographic negatives and diapositives, since a mask, negative, or diapositive of such types as figured, silvered or aluminized plates might be employed.

The diapositive of the figure is then placed in proper relation with the silvered and light sensitive transparent coated glass for exposure to a light of high intensity for the purpose of pro-

jecting the image to the coating. A strong actinic light which may be produced by an arc lamp may be employed with an exposure having a duration of about thirty seconds. In placing the image from the diapositive, or mask, with respect to the light sensitive coating on the glass, we find it preferable to cut the diapositive to substantially the same diameter as the reticle and with the image properly oriented to employ a ring as a frame to hold the negative and reticle in position. A considerable number of reticles may be exposed at a time. The exposure must be of sufficient duration and intensity to cause the proper reaction by the exposed light sensitive coating.

After the light sensitive coating of the reticle has been exposed under the diapositive to light of strong actinic intensity the coated surface of the reticle is washed to develop the enamel resist. The developer may consist of alcohol particularly where a resin type colloid is employed, or of water where an albumen or glue colloid is used. Likewise, a methyl violet dye, or other dye, may be mixed with the developer to dye the cold top image so that it may more readily be seen. The reticles are lifted from the developer following an immersion of about ten seconds and permitted to drain. As soon as the image is clearly seen the reticles are rinsed in water and dried. The portion of the light sensitive coating that is exposed to the light and rendered insoluble in the developer fluid, forms an enamel resist to protect the under coat of silver in the subsequent silver etching process. That portion of the coating protected from the light by the negative is dissolved away leaving the image contained in the unprotected silver coating. In this development process if the protective coating is weak and tends to come off in the developer an underexposed condition is indicated, and if the image does not raise an overexposed condition is indicated.

The development is completed by washing in water and by lightly stroking the surface with a wad of cotton or a soft brush. A well known hardening solution may be employed to prevent any tendency of the enamel coating to blister. The application of heat in drying may likewise serve to harden the enamel for better withstand-  
ing the action of the etching mordant.

The silver in the image which is unprotected by the enamel is etched or dissolved away by immersing the reticles in a solution of the well known Farmer's reducer, containing sodium thiosulphate and potassium ferricyanide, although other known agents may be employed. This solution does not attack the Cold Top or other enamel resist and this step of the process is terminated by complete transparency of the image on the exposed glass. Completion of this step may be accomplished in about one minute following which the reticles are rinsed and dried.

The etching of the glass is preferably accomplished by exposing the reticles to hydrofluoric acid fumes. This etching mordant will attack the Cold Top or other light sensitive enamel and the effective resist is formed by the undercoat-  
ing of silver. It is found that a four or five second exposure of the reticles to fumes of commercial fifty-two percent acid, heated in a water bath to a temperature of 120° F. will produce the desired etching of the glass. To maintain uniform strength of the acid fumes a lead container may be employed, having a sliding cover on one side of which is a recess for holding the reticle and an opening therein to expose the image.

The reticle is placed over the recess and the cover is moved over the container for the required time, whereupon the reticle is removed and placed in water to check the etching action.

A rinse of concentrated nitric acid, or other known solution, is applied to the reticle for the removal of the silver and remaining enamel.

The etched glass is then washed, dried and filled in any well known manner, to enable the image to properly stand out, and thus complete the production of the reticle in accordance with the practice of our invention.

Our process may also be applied to etching of plastic materials, using a suitable organic solvent in place of the hydrofluoric acid, and some minor modifications in cleaning, etc., which will be obvious to those skilled in the art. For example, a cellulose acetate sheet might be coated with silver and light sensitive colloid and exposed and developed as described, leaving the silver film as a resist, and the figure etched in the cellulose acetate surface with acetone.

The application of our invention to the pro-

duction of reticles as disclosed above is intended to be merely illustrative. Other variations and applications of the invention will readily occur to those skilled in the art. Therefore, our invention should be limited only in accordance with the scope of the appended claim.

We claim as our invention:

A process for photographically applying an image to an article of glass or similar material, comprising, successively applying a plurality of layers of silver coating to said article until the metallic surface has a slightly white appearance, successively applying a plurality of layers of light sensitive coating to said silver coating until said coating has assumed a thickness substantially equal to one-half the wave length of red light, projecting an image of the desired configuration upon said light sensitive coating, and then developing said coating to remove that portion of the light sensitive coating conforming to the configuration of the image projected thereon.

JOHN V. SIGFORD.  
WALDO H. KLINEVER.